

Dec. 23, 1958

A. H. JAFFEY ET AL  
METHOD OF SEPARATING URANIUM, PLUTONIUM AND FISSION  
PRODUCTS BY BROMINATION AND DISTILLATION  
Filed Jan. 8, 1947

2,865,704



INVENTORS.  
Arthur H. Jaffey  
Glenn T. Seaborg

BY

Roland A. Anderson  
Attorney.

1

2,865,704

## METHOD OF SEPARATING URANIUM, PLUTONIUM, AND FISSION PRODUCTS BY BROMINATION AND DISTILLATION

Arthur H. Jaffey, Chicago, Ill., and Glenn T. Seaborg, Albany, Calif., assignors to the United States of America as represented by the United States Atomic Energy Commission

Application January 8, 1947, Serial No. 720,920

7 Claims. (Cl. 23—14.5)

This invention relates to the treatment of compositions containing element 94 and more particularly relates to reaction and volatilization methods for separating element 94 and foreign products such as fission products and uranium from each other.

In this specification and claims the name of the element, unless otherwise indicated, designates generically the element either in its free or combined state. The designation "plutonium" or "element 94" as used throughout the present description refers to the transuranic element having an atomic number of 94. The expression "94<sup>239</sup>" means the isotope of element 94 having an atomic weight or mass of 239. Similarly, the terms "element 93" or "neptunium" refer to the transuranic element having an atomic number of 93.

It is now known that the transuranic elements 94 and 93 and also elements of lower atomic weight known as fission products may be produced by the bombardment of uranium metal or uranium compounds with neutrons. Natural uranium contains a large proportion of the isotope U<sup>238</sup> and a smaller proportion (about 1/139 of 238) of the isotope U<sup>235</sup>. The reaction of U<sup>238</sup> with slow neutrons produces the isotope U<sup>239</sup> which undergoes beta decay, with a half-life of 23 minutes, to 93<sup>239</sup> which in turn decays with a half-life of 2.3 days to 94<sup>239</sup>.

The slow neutrons also react with U<sup>235</sup> to produce nuclear fission and two fragments called fission fragments. These fission fragments are in general highly radioactive, and undergo beta disintegration with gamma radiation into chains of two groups, a light group of elements with atomic numbers from approximately 35 to 44 and a heavy group with atomic numbers from approximately 51 to 58. These elements either alone or combined as compounds are known as fission products.

The half-lives of the various intermediate nuclei of these fission products range from fractions of a second to a year or more with several of the important species having half-lives of the order of a month or so. The dangerous radioactivity of fission products having a very short half-life may be eliminated by suitable aging of a few days. This aging period also serves to permit the transformation of the greater part of the 92<sup>239</sup> to 93<sup>239</sup>, and of the 93<sup>239</sup> into 94<sup>239</sup>. The fission products of very long half-lives have a minimum of radioactivity, but the fission fragments of intermediate half-lives, of the order of a month or so, for example: Sr<sup>89</sup>, U (57-day half-life), Zr, Cb, and Ru of the group of atomic numbers from 35 to 44; and Te<sup>127</sup>, Te<sup>129</sup>, I<sup>131</sup>, Xe<sup>133</sup>, Ba (12 days' half-life), La<sup>140</sup>, and Ce of 20-day and 200-day half-lives, from the group of atomic numbers from 51 to 58 inclusive, make the mass extremely difficult to handle without danger of exposure of personnel to gamma radiation.

In the production of plutonium by the bombardment of natural uranium with neutrons produced by a chain

2

reaction in a uranium lattice reactor, the reaction is usually stopped when the concentration of the plutonium is still very small in relation to the U<sup>238</sup>, usually less than 1 percent by weight and often less than one or several parts per million parts of U<sup>238</sup>. Consequently the percentage of fission products is also very small, for example of the order of 0.02 percent of the mass by weight. The separation of the plutonium from the mass of uranium and from the fission products is therefore a very difficult process, not only because of the extremely minute concentrations, but also because of the dangerous radioactivity of the fission products present. The concentration and separation of plutonium from the radioactive fission products and uranium may be accomplished by the process of this invention.

As noted above, the very short half-life of neptunium (2.3 days) makes the chemical separation of neptunium from plutonium unnecessary since by suitable aging neptunium decays with beta emission to form plutonium.

10 The reaction of the uranium with neutrons may be carried out at such a slow rate of disintegration that a large proportion of neptunium decays to plutonium during the course of the reaction in the neutronic reactor, or the mass as removed from the neutronic reactor may be stored for a few days after the reaction to increase the 94 present in the mass, and ultimately all of the 93 present will be converted to 94 by radioactive decay.

15 An object of this invention is to provide a simple and efficient method of separating plutonium from uranium and radioactive fission products.

20 A further object of this invention is to provide a method of producing a pure and relatively non-corrosive plutonium halide suitable for use in the bomb reduction method of plutonium metal production.

25 An additional object of this invention is to provide a method for the selective separation of contaminating elements from plutonium, whereby individual, or groups of, contaminants may be separated from plutonium in a single cycle of operations.

30 Other objects and advantages of this invention will become apparent as the following detailed description progresses.

35 This invention is broadly a process for the separation of plutonium from uranium and fission products, which comprises the bromination of a mass consisting of plutonium and contaminants, the separation of contaminants which form more volatile bromides than plutonium bromide by the volatilization of the bromides of these contaminants from the plutonium, and the separation of plutonium from contaminants which form less volatile bromides by the volatilization of plutonium bromide from these less volatile bromides. Thus by the process 40 of this invention plutonium can be separated from uranium and other contaminants and a substantially pure plutonium bromide obtained.

45 The volatilities of uranium, plutonium and the various fission products and of their bromides have been tabulated in Table I.

50 Temperatures are given for four vapor pressures, 10<sup>-4</sup>, 10<sup>-3</sup>, 10<sup>-2</sup> and 1 atmospheres. Thus T<sub>10<sup>-4</sup></sub>, T<sub>10<sup>-3</sup></sub>, T<sub>10<sup>-2</sup></sub> and T<sub>1</sub> are the temperatures in degrees Kelvin at which the partial pressures 10<sup>-4</sup>, 10<sup>-3</sup>, 10<sup>-2</sup> and 1 atmospheres respectively are obtained. These pressures are partial pressures of the species listed and are total pressures only when the species listed is the only gaseous species above the condensed phase.

55 Estimated values and ones obtained by extrapolation from experimental data are given in parentheses.

3  
*Table I*

| At. No.           | Element    | T <sub>b</sub> , Boiling Point at P atmospheres,<br>°Kelvin |                   |                   |                |
|-------------------|------------|-------------------------------------------------------------|-------------------|-------------------|----------------|
|                   |            | T <sub>10-4</sub>                                           | T <sub>10-3</sub> | T <sub>10-2</sub> | T <sub>1</sub> |
| 35                | Bromine    |                                                             |                   |                   | 331.8          |
| 36                | Krypton    |                                                             |                   |                   | 120.1          |
| 37                | Rubidium   | 496                                                         | 561               | 650               | 952            |
| 38                | Stroncium  | 900                                                         | 1,010             | 1,150             | 1,657          |
| 39                | Yttrium    | 2,100                                                       | 2,300             | 2,700             | 3,500          |
| 40                | Zirconium  | 2,450                                                       | 2,700             | 3,000             | 3,850          |
| 41                | Columbium  | 3,340                                                       | 3,700             | 4,120             | 5,400          |
| 42                | Molybdenum | 3,000                                                       | 3,330             | 3,750             | 5,077          |
| 43                | Masurium   | 3,000                                                       | 3,300             | 3,700             | 5,000          |
| 44                | Ruthenium  | 2,900                                                       | 3,180             | 3,500             | 4,500          |
| 51                | Antimony   | 1,025                                                       | 1,160             | 1,340             | 1,890          |
| 52                | Tellurium  | 758                                                         | 825               | 907               | 1,130          |
| 53                | Iodine     | 282                                                         | 308               | 341               | 456            |
| 54                | Xenon      |                                                             |                   |                   | 165            |
| 55                | Caesium    | 476                                                         | 544               | 634               | 963            |
| 56                | Barium     | 985                                                         | 1,116             | 1,293             | 1,911          |
| 57                | Lanthanum  | 1,800                                                       | 2,000             | 2,250             | 3,000          |
| 58                | Cerium     | 1,700                                                       | 1,850             | 2,100             | 2,800          |
| 92                | Uranium    | 2,350                                                       | 2,580             | 2,900             | (3,800)        |
| 94                | Plutonium  | 1,950                                                       | 2,200             | 2,500             | 3,508          |
| Bromides          |            |                                                             |                   |                   |                |
| RbBr              | (935)      | 1,039                                                       | 1,176             | 1,625             |                |
| SrBr <sub>2</sub> | (1,300)    | plus or minus 100°                                          |                   | 2,150             |                |
| YBr <sub>3</sub>  | (1,050)    | (1,150)                                                     | (1,300)           | (1,740)           |                |
| ZrBr <sub>2</sub> | (900)      | plus or minus 200°                                          |                   | (1,500)           |                |
| ZrBr <sub>3</sub> | (1,050)    | plus or minus 200°                                          |                   | Disproportionates |                |
| ZrBr <sub>4</sub> |            |                                                             |                   |                   |                |
| ObBr <sub>3</sub> | 422        | 477                                                         | 518               | 630               |                |
| MoBr <sub>4</sub> | (370)      |                                                             | (430)             | 545               |                |
| RuBr <sub>3</sub> |            | Plus or minus 100°                                          |                   | (620)             |                |
| SbBr <sub>3</sub> | (380)      | (360)                                                       | (408)             | (1,200)           |                |
| TeBr <sub>2</sub> |            |                                                             |                   | 561               |                |
| TeBr <sub>4</sub> |            |                                                             | (610)             | 612               |                |
| IBr               | (245)      | (270)                                                       | 298               | (820)             |                |
| CsBr              | (905)      | 1,007                                                       | 1,139             | 1,573             |                |
| BaBr <sub>2</sub> | (1,250)    | plus or minus 100°                                          |                   | (2,100)           |                |
| LaBr <sub>3</sub> | (1,110)    | (1,220)                                                     | (1,360)           | (1,850)           |                |
| CeBr <sub>3</sub> | (1,100)    | (1,210)                                                     | (1,350)           | (1,830)           |                |
| UBr <sub>3</sub>  | 1,120      | 1,240                                                       | 1,380             | (1,840)           |                |
| UBr <sub>4</sub>  | 680        | 740                                                         | 800               | 1,060             |                |
| PuBr <sub>3</sub> | 1,085      | 1,190                                                       | 1,335             | 1,785             |                |

The vapor pressures of YBr<sub>3</sub>, UBr<sub>4</sub> and PuBr<sub>3</sub> over the range of temperatures and pressures shown by Table I are graphically portrayed in the sole figure.

In accordance with one embodiment of this invention uranium metal, carbides, sulfides, oxides, peroxides or other compounds of uranium capable of reacting with the bromine or bromine derivatives to form uranium tetrabromide are irradiated with neutrons to obtain neptunium, plutonium and fission products, and the reaction is terminated while a substantial proportion of uranium remains unconverted. This mass is then aged to convert the neptunium to plutonium by nuclear disintegration. The mass is then treated with hydrogen bromide at an elevated temperature of, for example, the boiling point of YBr<sub>3</sub> at the pressure used. As this temperature is approached, the following radioactive fission products are volatilized from the mass unchanged: bromine, krypton, iodine and xenon. The bromination of the mass at this temperature and pressure will convert the following radioactive fission products to their respective bromides and they will be volatilized as shown in Table I and may be separated from the mass: RbBr, ZrBr<sub>4</sub>, CbBr<sub>5</sub>, MoBr<sub>4</sub>, RuBr<sub>3</sub>, SbBr<sub>3</sub>, TeBr<sub>2</sub>, TeBr<sub>4</sub>, CsBr, and YBr<sub>3</sub> and UBr<sub>4</sub>. It will be noted that both zirconium and uranium form several bromides with varying volatilities. Zirconium tetrabromide, however, volatilizes at 630° K. under atmospheric pressure. Similarly uranium tetrabromide volatilizes at 1060° K. under atmospheric pressure. By using an excess of hydrogen bromide the higher bromides of zirconium and uranium will be formed and will volatilize at these relatively low temperatures.

Any iodine remaining in the mass will be volatilized with the hydrogen bromide to form IBr, and thus may be separated from the mass.

After the above bromides are substantially removed by volatilization, the temperature may be raised to the boiling point of PuBr<sub>3</sub> and the bromination continued. In

70 this range of temperature PuBr<sub>3</sub> will form and vaporize from the remaining constituents of the mass. The constituents remaining should include BaBr<sub>2</sub>, SrBr<sub>2</sub>, LaBr<sub>3</sub>, CeBr<sub>3</sub> and any radioactive fragments which do not form bromides. It is believed that this would include masurium since no masurium bromides are known and masurium has not been detected in the portions volatile at the above temperatures.

It may be desirable to broaden the PuBr<sub>3</sub> fraction in the first cycle of vaporization so that it will include YBr<sub>3</sub>, LaBr<sub>3</sub>, and CeBr<sub>3</sub>, and this fraction can then be revolatilized with hydrogen bromide, and by suitable adjustment of the temperatures and pressures and volatilization through several cycles, the plutonium may be effectively separated from this fraction to yield substantially pure PuBr<sub>3</sub>. It is also contemplated that other methods of separation may be used to separate the radioactive fission products which form bromides with boiling points closest to that of PuBr<sub>3</sub>. Thus Y, La, and Ce may be separated by adsorption or precipitation methods either before or after the separation of Pu from the other contaminants by the process of this invention.

It will be noted that the separation of plutonium by the process of this invention has certain great advantages over other types of separation. Thus the radioactive fission products such as Xe, Kr, Br, and I, which volatilize or form bromides with low boiling points, are separated quantitatively by a single volatilization step. Uranium, which forms the great bulk of a neutron-irradiated mass, may be very effectively separated from plutonium since the boiling point of uranium tetrabromide is 725° C. lower than that of plutonium tribromide. And in addition, those radioactive fission products which are heavy gamma ray emitters, such as Zr, Cb, Cs, and Ba, form bromides with volatilities greatly different from plutonium bromide and so may be easily separated from plutonium by volatilization of the bromides.

Although the process of this invention may be carried out at atmospheric pressure, it is to be understood that this process may also be carried out at greater or less than atmospheric pressure by suitable adjustment of the temperatures used, as shown in Table I. Desirable changes in the temperatures and pressures involved in the use of brominating agents other than hydrogen bromide are also contemplated.

It will be understood that where a compound of uranium is irradiated which is not converted to the tetrabromide by treatment with hydrogen bromide, uranium and other compounds obtained after irradiation may be converted to compounds which are convertible to bromides. Thus uranium nitrate may be converted to the oxide by heating and the oxide reacted with hydrogen bromide. Uranium metal, although it may be directly treated with hydrogen bromide, can be heated with oxygen to form U<sub>3</sub>O<sub>8</sub> which may be reduced to UO<sub>2</sub> with hydrogen. This compound can then readily be converted to UBr<sub>4</sub> by treatment with hydrogen bromide.

It is not necessary that the treatment with hydrogen bromide be with anhydrous hydrogen bromide at elevated temperatures, although this is preferable since it then removes volatile radioactive fission products in the initial stage of the process. The treatment with hydrogen bromide may be with an aqueous solution of hydrogen bromide to obtain UBr<sub>4</sub> which may then be volatilized as set forth above.

Although the process of this invention may be used as a complete method for the separation of plutonium from uranium and radioactive fission products, it also may be conveniently used for the concentration and/or separation of plutonium from uranium or from radioactive fission products. Thus the bromination and volatilization of plutonium, uranium and radioactive fission product contaminants, either individually or in any suitable combination, may be used as a separate step in any other plutonium separation process.

In accordance with another embodiment of this invention, neutron-irradiated uranium may be treated with bromine to separate plutonium from uranium. Thus when metallic uranium and plutonium are treated with bromine, the reactions are believed to proceed in the following manner:



and



The bromine may be passed over the mass containing uranium and plutonium at a temperature of approximately  $300^\circ \text{ C.}$  and the uranium tetrabromide which forms may be volatilized away and condensed as a distillate to separate the uranium from the plutonium. This may be repeated as often as necessary to increase the ratio of separation.

In another embodiment of this invention and one which has been found to be a preferable method for separating plutonium from uranium, the oxides of plutonium and uranium may be reacted with hydrogen bromide to form their respective bromides and these separated by a fractional distillation. The reactions of these oxides are believed to be the following:



An experiment was carried out with this method in which samples of plutonium and of uranium were mounted on platinum, ignited to redness and then counted. The samples were then placed in a suitable apparatus and treated with hydrogen bromide at various temperatures for 30 minutes, removed and again counted. Numerous runs were made at each temperature; the results are summarized in Table II.

Table II

| Temperature, $^\circ\text{C.}$ | Pu volatilized in 30 minutes, Percent | U volatilized in 30 minutes, Percent |
|--------------------------------|---------------------------------------|--------------------------------------|
| 300                            |                                       | 5                                    |
| 400                            |                                       | 72                                   |
| 500                            | 15                                    |                                      |
| 600                            | 33                                    | 85                                   |
| 700                            | 90                                    | 95                                   |

A variation of the bromination of the oxides of uranium and plutonium is a method whereby the oxides are mixed with excess carbon and heated to red heat. A stream of  $\text{N}_2$  or other inert gas is bubbled through  $\text{Br}_2$  and passed over the mixture. The resulting plutonium and uranium bromides may then be fractionally separated by condensation. This type of separation may be illustrated by the following reactions:



and



or



There are numerous other brominating agents which may be used in the process of this invention as well as bromine and hydrogen bromide which have been described above. For instance, an effective brominating agent has been found to be a sulphur bromine mixture, as shown in the following reactions:



and



The following is an example of this method of bromination it being understood that it is given only for purposes of illustration and that it is not intended to limit the invention to the details given in the experiment.

Bromine vapor at ca. 100 mm. pressure was passed

over sulphur at  $120^\circ \text{ C.}$  The bromine dissolved in the sulphur to form red liquid sulphur bromide. The bromine-sulphur bromide mixture was passed through a quartz reaction tube containing the  $\text{PuO}_{2-x}\text{H}_2\text{O}$  at  $800^\circ \text{ C.}$  The flow rate of the bromide was controlled at approximately 5 cc. per minute by a capillary at the outlet end of the system leading to a vacuum apparatus. Over a period of several hours 10 milligrams of Pu as  $\text{PuO}_{2-x}\text{H}_2\text{O}$  was converted to a green sublimate of  $\text{PuBr}_3$  which condensed at the outlet end of the reactor. The free energy of the reaction was calculated to be

$$F_{1000^\circ\text{K.}} = -34 \text{ K. cals.}$$

indicating that the sulphur-bromine mixture is more effective than HBr as the brominating agent. Phosphorus pentabromide, phosphorus tribromide, aluminum bromide, antimony pentabromide, and antimony tribromide can also be used. The following equations serve to illustrate reactions involving several of these brominating agents:



The end product produced by the process of this invention, anhydrous plutonium tribromide, is a blue-green crystalline compound having the following properties:

Melting point— $654^\circ \text{ C.} \pm 4^\circ$

Crystalline structure:

Orthorhombic

Four molecules per unit cell

Lattice constants—

$$a_1 = 12.57 \pm 0.05 \text{ A.}$$

$$a_2 = 4.11 \pm 0.03 \text{ A.}$$

$$a_3 = 9.13 \pm 0.04 \text{ A.}$$

Calculated density—6.69

Experiments have been carried out to determine if plutonium forms bromides other than that of the trivalent plutonium, but it is believed from the results of these experiments that plutonium tribromide is the only one formed in reactions involving anhydrous reactants.

While there have been described certain embodiments of our invention, it is to be understood that it is capable of many modifications, and changes therefore may be made without departing from the spirit and scope of the invention as described in the appended claims in which it is the intention to claim all novelties and invention as broadly as possible in view of the prior art.

What is claimed is:

1. The method of separating plutonium from uranium and radioactive fission products, which comprises reacting a neutron-irradiated uranium mass with a brominating agent at an elevated temperature to form the bromides of uranium, plutonium and such fission products as form bromides, distilling the uranium bromide, volatile fission products, and volatile fission product bromides from the mass by subjecting the mass to a temperature between  $777^\circ$  and  $1467^\circ \text{ C.}$  and a pressure substantially equal to the vapor pressure of  $\text{YBr}_3$  at said temperature and then distilling the plutonium bromide from the mass by subjecting the mass to a temperature greater than  $1512^\circ \text{ C.}$  and pressure less than the vapor pressure of  $\text{PuBr}_3$  at that temperature, and separately collecting the resulting distillate.
2. The process of claim 1 wherein the brominating agent is bromine.
3. The process of claim 1 wherein the brominating agent is hydrogen bromide.
4. The process of claim 1 wherein the brominating agent is  $\text{AlBr}_3$ .
5. The process of claim 1 wherein the brominating agent is a mixture of sulfur and bromine.
6. The method of separating  $\text{PuBr}_3$  and  $\text{UBr}_4$ , which

comprises distilling the  $U\text{Br}_4$  from a mixture of  $\text{PuBr}_3$  and  $U\text{Br}_4$  by subjecting the mixture to a temperature higher than  $392^\circ \text{ C}$ . and pressure less than the vapor pressure of  $U\text{Br}_4$  at said temperature, and then distilling the plutonium bromide from the mass by subjecting the mass to a temperature higher than  $812^\circ \text{ C}$ . and pressure less than the vapor pressure of  $\text{PuBr}_3$  at said temperature, and separately collecting the distillate.

7. A method of separating uranium and plutonium from neutron-irradiated uranium mass, which comprises treating said mass with hydrogen bromide at a tempera-

ture of approximately  $400^\circ \text{ C}$ . and pressure of approximately  $10^{-4}$  atmospheres whereby  $U\text{Br}_4$  is vaporized from the mass, selectively condensing said  $U\text{Br}_4$  vapor, heating said neutron-irradiated mass to approximately  $700^\circ \text{ C}$ . under a pressure of  $10^{-4}$  atmospheres, and selectively condensing the  $\text{PuBr}_3$  vapor thus formed.

References Cited in the file of this patent

UNITED STATES PATENTS

1,434,485 D'Adrian \_\_\_\_\_ Nov. 7, 1922